

## UNITED STATES PATENT OFFICE

2,445,632

INDIGOSOL COMPOSITION COMPRISING A  
NAPHTHOL SULFONATE AND METHOD OF  
APPLYING SAMEEarl L. Pelton and Charles O. Hutschenreuther,  
Midland, Mich., assignors to The Dow Chemical  
Company, Midland, Mich., a corporation of  
DelawareNo Drawing. Application October 5, 1945,  
Serial No. 620,624

15 Claims. (Cl. 8—70)

1

This invention concerns certain new compositions comprising, as essential ingredients, an Indigosol derived from tetrabromindigo together with an agent for facilitating development, i. e. hydrolysis and oxidation, of the Indigosol to the colored form of tetrabromindigo. It pertains especially to powders and pastes comprising said essential ingredients, which powders and pastes are adapted for use in the dyeing and printing of textile fibers and fabrics. It pertains more particularly to such pastes which, when supplemented by usual Indigosol-printing aids, e. g. an oxidizing agent and a printing gum or other thickener, are adapted for use in fabric printing processes which involve development of the dyestuff on the fabric by steaming of the latter. The invention also concerns a method of printing fabrics and the like with the new compositions and developing the dyestuff color by steaming.

The dyestuffs known as "Indigosols," i. e. acid-sulphate esters of the leuco form of indigoid dyes, are, when in the form of their alkali salts, sufficiently stable for storage and shipment. They are used extensively for the dyeing and printing of fabrics. Use of the Indigosols permits the dyer to avoid a step of reducing the usual oxidized form of the corresponding indigoid vat dye. Also, the Indigosols may be applied to fabrics in conjunction with other dyestuffs, e. g. azo dyes, to obtain desired color combinations.

After application of an Indigosol to a fabric, the color of the corresponding indigoid vat dye is developed by hydrolysis and oxidation of the Indigosol, usually under acidic conditions and in the presence of an oxidizing agent such as sodium or potassium nitrite, chloride, or bichromate, etc. Development may be accomplished by immersion in an aqueous bath containing the developing agents, or it may be accomplished by steaming under acidic conditions of a fabric which has been treated with a mixture comprising an Indigosol and an oxidizing agent.

For printing purposes, particularly the printing of fabrics in a continuous manner, development by steaming is most convenient and economical and is preferred when it may satisfactorily be employed. However, Indigosols are known to vary widely as regards the readiness with which they undergo development to the colored form of the corresponding indigoid vat dye, and steaming is less effective than immersion in a developing bath in causing development of the Indigosols which are resistant to hydrolysis and oxidation. Accordingly, although most, if not all, Indigosols may satisfactorily be used in dye-

2

ing and printing processes wherein development is accomplished by immersion in a bath, certain Indigosols, including those with which this invention is concerned, have not heretofore been adapted for use in processes involving development of the dyestuff by steaming. For instance, Christ, J. Soc. Dyers and Colourists, 54, 94 (1938), in a table indicating the relative ease with which various Indigosols undergo development, terms Indigosol O4B (i. e. the sodium acid-sulphate ester of leuco 5,7,5',7'-tetrabromindigo) "inert." In this publication, the Indigosols were presumably developed by steaming, since Indigosol O4B does not develop readily under usual steaming conditions, but is readily developed by immersion in an acidic developing bath.

We have discovered that an Indigosol derived from tetrabromindigo, e. g. Indigosol O4B, may be caused to develop readily in a steaming operation by admixing one or more of certain naphthol sulphonic acids, or salts thereof, with the Indigosol prior to the steaming operation. The naphthol sulphonic acids which we have found to be effective for the purpose are 1-naphthol-2-sulphonic acid, 1-naphthol-4-sulphonic acid and 2-naphthol-7-sulphonic acid. A number of other naphthol mono- and di-sulphonic acids were similarly tested, but were found to have relatively little, or no, action in accelerating development of the dyestuff.

The compositions provided by the invention are powders, or pastes, which comprise as essential ingredients a salt of an Indigosol derived from tetrabromindigo, preferably 5,7,5',7'-tetrabromindigo, and a salt of one or more of the above-mentioned naphthol sulphonic acids which are effective in promoting development of the dyestuff to its colored form. Usually, a minor amount of an alkali, e. g. sodium or potassium carbonate, is also added further to stabilize the Indigosol during storage and shipment. The Indigosol and naphthol sulphonic acid are usually employed in the form of alkali salts thereof, e. g. sodium or potassium salts, but other salts such as alkanolamine salts of the compounds may be used.

The naphthol sulphonate is somewhat effective in increasing the readiness with which the Indigosol may be developed, regardless of the proportion in which it is used but, for use in printing operations in which the color is to be developed by steaming, it is advantageously employed in amount corresponding to between 3 and 20 per cent of the weight of the Indigosol. However, it

may be used in smaller proportions or in as great a proportion as desired.

Mixtures comprising the Indigosol and naphthol sulphonate are more stable against chemical change during storage when in the form of powders than when converted to pastes. Accordingly, the mixtures may advantageously be marketed in powder form and the powder may be used in forming a paste shortly prior to employment of the latter, e. g. in a printing operation. In addition to the ingredients mentioned above, the powders may, if desired, comprise one or more other ingredients such as urea, sodium chloride, ammonium chloride, sodium sulphate, dextrose, sugar, sodium benzene sulphonate, or starch, etc., but these are not required.

The powder is usually prepared so to contain between 20 and 80 per cent of the Indigosol salt, based on the anhydrous weight of all solid ingredients, but it may contain the Indigosol in proportions smaller or greater than those just given.

A powder prepared as just described is suitable for dyeing or printing purposes and is particularly adapted for use in printing operations wherein the color is to be developed by steaming of the printed fabric. During, or prior to, use of the composition for such purposes certain other agents such as an oxidizing agent, an acid, and, for printing purposes, a printing gum are admixed therewith, but such further agents are usually added by the dyer in amounts and under conditions which meet his particular need.

For instance, a printing paste may be prepared by admixing, with the powder, an oxidizing agent, such as sodium or potassium chlorate, chromate, or dichromate, etc., in amount sufficient to oxidize the leuco dyestuff corresponding to the Indigosol, a liquid medium such as water, alcohol, or glycerine, etc., and a printing gum, e. g. British gum or gum tragacanth, etc. The oxidizing agent is usually employed in considerable excess over the amount just stated. Other usual printing aids such as starch, dextrose, sugar, urea, or salts such as sodium chloride, ammonium chloride, or sodium sulphate, etc., may also be added. Although the ingredients of such paste may be admixed in any desired manner, or order, the paste is conveniently prepared by dissolving the Indigosol salt, naphthol sulphonate, oxidizing agent and any other soluble solid ingredients other than the thickening agent in hot water, e. g. water heated to from 60° to 100° C. or above, and thereafter adding with stirring an aqueous paste of starch and a printing gum in the amount necessary to form a final printing paste of the body or thickness which is desired.

In addition, to the ingredients just mentioned, a non-acidic substance which, on being heated, will generate an acid may be incorporated in the printing paste so that the latter, after being applied to a fabric, may be developed merely by treatment with steam. A number of acid-acting substances such as ammonium sulpho-cyanide and diethyl tartrate are known to the art. Usually, instead of incorporating such acid-acting substance in the paste in amount sufficient to render the latter acidic when heated, the acid-acting substance is omitted from the paste and a fabric printed with the latter is treated with acid prior to or during steaming of the printed goods.

Fabrics of cotton, wool or rayon, etc., are printed in conventional manner with the printing paste, after which the characteristic blue color

of tetrabromindigo is developed on the fabric either by immersing the latter in a slightly acid aqueous developing bath, or by steaming in the presence of an acid. The color is preferably developed by contacting the goods with a vapor mixture of steam and a volatile carboxylic acid, e. g. formic, acetic or propionic acid or a mixture of such acids. Alternatively, the printed fabric may, if desired, be wetted or moistened with a dilute solution of any desired acid and thereafter be steamed. When using the printing pastes provided by the invention, the time of steaming required for development of the blue color of tetrabromindigo is usually in the order of from 2 to 10 minutes. After developing the color of the print, the fabric is washed and dried.

The following example describes certain ways in which the principle of the invention has been applied; but it not to be construed as limiting its scope.

#### Example

In each of a series of experiments, 50 parts by weight of Indigosol O4B of between 83.5 and 85.5 per cent concentration (the remainder being salts such as sodium chloride, sodium carbonate, sodium sulphate, etc.) was intimately admixed with the sodium naphthol sulphonate named in the following table in the amount also given and also with between 22.5 and 24.3 parts of water-soluble dextrose. The resultant powder was used in preparing a printing paste as follows: Three parts by weight of the Indigosol-containing powder, 5 parts of urea, 4 parts of sodium chromate and 1 part of ammonium chloride were dissolved in 27 parts of water which had been preheated to a temperature in the order of from 60° to 90° C. The solution was converted to a paste by adding, with stirring, 60 parts by weight of a stiff aqueous paste composed of approximately 91.75 per cent by weight water, 5 per cent corn starch, 3 per cent gum tragacanth and 0.25 per cent stearic acid. Cotton cloth was printed with the paste thus prepared and was thereafter exposed for about 6 minutes to a vapor mixture of steam, formic acid and acetic acid which was formed by passing steam first through a bath composed of approximately 2 molecular equivalents of formic acid and one molecular equivalent of acetic acid and thence into a chamber containing the printed cloth. After steaming the cloth, the latter was washed in soapy water, rinsed, dried and inspected to determine the quality of colored print obtained. The following table names the sodium naphthol sulphonate employed in each experiment, gives the proportion thereof as per cent of the weight of the Indigosol O4B in the printing paste and states the quality of color development on the print for each experiment.

| Run No. | Naphthol Sulphonate        |         | Color Development                           |
|---------|----------------------------|---------|---------------------------------------------|
|         | Kind                       | Percent |                                             |
| 65 1    | None                       | 0       | Very weak development.                      |
| 2       | Na 1-naphthol-2-sulphonate | 7.5     | Excellent; apparently complete and uniform. |
| 3       | Na 1-naphthol-4-sulphonate | 7.5     | Do.                                         |
| 4       | do                         | 11.3    | Do.                                         |
| 5       | Na 2-naphthol-7-sulphonate | 7.5     | Excellent and uniform.                      |
| 70 6    | do                         | 11.3    | Do.                                         |

Other modes of applying the principle of the invention may be employed instead of those explained, change being made as regards the method or compositions herein disclosed, provided the

steps or ingredients stated by any of the following claims or the equivalent of such stated steps or ingredients be employed.

We therefore particularly point out and distinctly claim as our invention:

1. A composition for coloring fabrics, which composition comprises as essential ingredients a salt of an acid-sulfate ester of a leuco dyestuff derived from tetrabromindigo and a salt of a naphthol sulphonic acid selected from the class consisting of 1-naphthol-2-sulphonic acid, 1-naphthol-4-sulphonic acid and 2-naphthol-7-sulphonic acid.

2. A composition for coloring fabrics, which composition comprises as essential ingredients an alkali metal acid-sulphate ester of the leuco form of 5,7,5',7'-tetrabromindigo and an alkali metal salt of a naphthol sulphonic acid selected from the class consisting of 1-naphthol-2-sulphonic acid, 1-naphthol-4-sulphonic acid and 2-naphthol-7-sulphonic acid, the naphthol sulphonate being present in amount corresponding to at least 3 per cent of the weight of the alkali metal acid-sulphate ester of leuco 5,7,5',7'-tetrabromindigo.

3. A composition for coloring fabrics, which composition comprises as essential ingredients a sodium acid-sulphate ester of the leuco form of 5,7,5',7'-tetrabromindigo and a sodium salt of a naphthol sulphonic acid selected from the class consisting of 1-naphthol-2-sulphonic acid, 1-naphthol-4-sulphonic acid, and 2-naphthol-7-sulphonic acid, the naphthol sulphonate being present in amount corresponding to between 3 and 20 per cent of the weight of the sodium acid sulphate ester of leuco 5,7,5',7'-tetrabromindigo.

4. A composition as defined in claim 1, when in the form of a powder.

5. A composition as defined in claim 2, when in the form of a powder.

6. A composition as defined in claim 3, when in the form of a powder.

7. A paste comprising the composition defined by claim 1 and intimately admixed therewith an aqueous medium and a thickening agent.

8. A paste comprising the composition defined by claim 2 and intimately admixed therewith an aqueous medium and a thickening agent.

9. A paste comprising the composition defined by claim 3 and intimately admixed therewith an aqueous medium and a thickening agent.

10. A printing paste comprising a salt of an acid-sulfate ester of a leuco dyestuff derived from tetrabromindigo, a salt of a naphthol sulphonic acid selected from the class consisting of 1-naphthol-2-sulphonic acid, 1-naphthol-4-sulphonic acid and 2-naphthol-7-sulphonic acid, an oxidizing agent, an aqueous medium, and a thickening agent.

11. A printing paste which comprises an alkali metal acid-sulphate ester of the leuco form of 5,7,5',7'-tetrabromindigo, an alkali metal salt of a naphthol sulphonic acid selected from the class consisting of 1-naphthol-2-sulphonic acid, 1-

naphthol-4-sulphonic acid, and 2-naphthol-7-sulphonic acid, an oxidizing agent, a printing gum, and an aqueous medium.

12. A printing paste which comprises an alkali metal acid-sulphate ester of the leuco form of 5,7,5',7'-tetrabromindigo, an alkali metal salt of a naphthol sulphonic acid selected from the class consisting of 1-naphthol-2-sulphonic acid, 1-naphthol-4-sulphonic acid, and 2-naphthol-7-sulphonic acid, an oxidizing agent in amount sufficient to oxidize the dyestuff during development of the latter, a printing gum, and water, the naphthol sulphonate being present in amount corresponding to at least 3 per cent of the weight of the alkali metal acid sulphate ester of the leuco 5,7,5',7'-tetrabromindigo.

13. A printing paste which comprises a sodium acid-sulphate ester of the leuco form of 5,7,5',7'-tetrabromindigo, a sodium salt of a naphthol sulphonic acid selected from the class consisting of 1-naphthol-2-sulphonic acid, 1-naphthol-4-sulphonic acid, and 2-naphthol-7-sulphonic acid, an oxidizing agent in amount sufficient to oxidize the dyestuff during development of the latter, a printing gum, and water, the naphthol sulphonate being present in amount corresponding to at least 3 per cent of the weight of the sodium acid sulphate ester of the leuco 5,7,5',7'-tetrabromindigo.

14. The process which comprises printing a fabric with a printing paste comprising a salt of an acid-sulfate ester of a leuco dyestuff derived from tetrabromindigo and a salt of a naphthol sulphonic acid selected from a class consisting of 1-naphthol-2-sulphonic acid, 1-naphthol-4-sulphonic acid and 2-naphthol-7-sulphonic acid, the naphthol sulphonate being present in amount corresponding to at least 3 per cent of the weight of the acid-sulfate ester of a leuco dyestuff.

15. The process which comprises printing a fabric with a printing paste comprising an alkali metal acid-sulphate ester of 5,7,5',7'-tetrabromindigo, an oxidizing agent in amount sufficient to oxidize the dyestuff during the development of the latter, an alkali metal salt of a naphthol sulphonic acid selected from the class consisting of 1-naphthol-2-sulphonic acid, 1-naphthol-4-sulphonic acid and 2-naphthol-7-sulphonic acid, the naphthol sulphonate being present in amount corresponding to between 3 and 20 per cent of the weight of the alkali metal acid sulphate ester of the leuco 5,7,5',7'-tetrabromindigo and thereafter acidifying and developing the dyestuff on the fabric by exposing the latter to steam.

EARL L. PELTON.

CHARLES O. HUTCHENREUTHER.

#### REFERENCES CITED

The following references are of record in the file of this patent:

#### UNITED STATES PATENTS

|           |          |                |
|-----------|----------|----------------|
| Number    | Name     | Date           |
| 2,173,824 | Chambers | Sept. 19, 1939 |